

# UNITED STATES PATENT OFFICE.

OTTO STEINER, OF CREFELD, GERMANY.

## PROCESS OF OBTAINING PURE TIN FROM CRUDE TIN OR TIN ALLOYS ELECTROLYTICALLY.

No. 890,249.

Specification of Letters Patent.

Patented June 9, 1908.

Application filed August 10, 1907. Serial No. 388,036.

To all whom it may concern:

Be it known that I, OTTO STEINER, subject of the Austrian Emperor, residing at Crefeld, Germany, have invented new and useful Improvements in Methods or Processes of Obtaining Pure Tin from Crude Tin or Tin Alloys Electrolytically, of which the following is a specification.

The present invention relates to a method 10 of refining tin electrolytically, particularly for extracting pure tin from alloys, wastages, residues etc. with the extraction of the foreign metals.

In the English patent specification No. 297 15 of the year 1895 (Claus), a method for refining tin electrolytically is described, consisting in tin alloys being subjected to electrolysis in an alkaline sulfur solution at a temperature of 90° C. and a current density of 1 20 ampere per square decimeter of electrode surface. Pure tin is precipitated at the cathode, whereas the impurities are deposited as sulfids and collect at the bottom of the bath. If, however, antimony and arsenic are 25 contained in the tin alloys which is employed as anode, these are deposited together with the tin at the cathode. If the tin is to be freed from these admixtures, the cathode deposit must be subjected to electrolysis a second 30 time in a solution of sodium thio-sulfate in hydrochloric acid.

In the practical execution of the method according to the present invention it has been found that is is possible in an alkaline 35 sulfur solution to obtain a compact metallic deposit of pure tin at the cathode in one single operation when the necessary precautions are observed.

Firstly, plates of pure tin or tin-plated 40 plates or sheets are employed as cathodes. On other metals, as iron, copper etc., the tin is precipitated spongy with generation of gas.

Secondly, care must be taken that the tension between the anode and cathode amounts 45 to less than 0.2 volt. If the tension between the electrodes exceeds this amount, a sudden rise of tension up to 0.6 volt and violent generation of gas or decomposition of the electrolyte takes place. That fact is caused by 50 sudden and violent evolution of hydrogen gas. See also the journal "Electrochemical and Metallurgical Industry" 1907, page 309. The previously metallic-bright cathode deposit becomes dull, sponge-like and oxidizes. 55 As the electrode tension is dependent on the

current density, of the concentration of the lye and of the distance between the electrodes, the tension may easily be kept below the critical limit of 0.2 volt by varying these components. When employing a 10% sulfid 60 of sodium solution as electrolyte and a distance between the electrodes of 1½ cm., current strengths up to ½ ampere per square decimeter of electrode surface can be employed without the tension reaching the 65 amount of 0.2 volt. If the proportion of sulfid of sodium in the electrolyte is increased, correspondingly higher strengths of current can be employed which is of great 70 importance commercially, for by raising the current density, the capacity of production of the apparatus is increased, and the duration of the electrolysis is shortened. In this manner the loss of tin from the tin which is employed in the plant, as well as the general 75 costs, is considerably diminished.

Further, before suspending fresh tin anodes having a bright metallic surface in the electrolyte, about 1% of the weight of the electrolyte of sulfur must be dissolved in the 80 same. This sulfur is preferably employed in the form of flowers of sulfur. It becomes precipitated as sulfid at the surface of the anodes and, acting thus as depolarizer, it enables the electrolysis to commence with 85 low tension. If the addition of sulfur is omitted before suspending new anodes, the crude tin anode behaves as an insoluble anode, and after closing the circuit the tension rises at once to 0.6 volt, violent generation of 90 gas and decomposition of the electrolyte takes place, but no tin is deposited. The cathodes become dull, and are then no longer usable for the further deposition of tin. The same electrolyte may be employed repeatedly 95 for electrolysis if sulfur is again added to the bath before suspending fresh anodes. The electrolyte can thus be kept for months in a condition fit for use.

Further, the electrolysis is to be carried 100 out so that the anode mud which is on the bottom of the bath and that which is attached to the anodes is not disturbed. In order to attain this all the operations must be carried out so that no violent movements 105 occur in the electrolyte. In this method, therefore, the lye cannot be circulated as in the electrolytic refining of copper. It is preferably heated indirectly by steam in each bath by itself and at the bottom of 110

each bath, whereby the lye is prevented at the same time from being decomposed by the electrolysis. After each electrolytic process the electrolyte is allowed to flow away very slowly through an overflow pipe placed above the bottom of the bath, whereupon the electrodes, together with the anode mud, are then removed and new electrodes suspended; the clear electrolyte is then allowed to flow in, 1% sulfur and so much sulfid of sodium are added that the original percentage of sulfid of sodium is produced again, and electrolysis is commenced again.

Lastly, care must be taken here also, as is generally usual, that the electrode-contacts of all the electrodes in a bath are made as good and uniform as possible. As only very low tension of 0.1 to 0.18 volt can be worked with in this method, small resistances are of much importance for the conduction of the current; with poor or non-uniform contacts the current is distributed very unequally to the individual electrodes of the bath which, besides the disadvantage of working unequally, also causes very different tensions between the individual anodes and cathodes of a bath, so that in many electrolytes only gas is generated, in others tin is deposited, and in others nothing takes place at all. Very uniform electrode contacts can be obtained in a quick and simple manner by soldering the electrodes directly to the homogeneous tinned conducting bars.

The illustrations Figures 1 to 5 on the accompanying drawing represent apparatus as is used for carrying the method in accordance with the present invention into practice. It is of course understood that these illustrations only represent one particular form of such apparatus, and that in practice all similar suitable apparatus can be employed if only they are similar in principle to the apparatus described hereafter.

In the drawing:—Fig. 1 is a vertical cross-section through the apparatus, one anode plate being seen in elevation; Fig. 2 shows a vertical cross-section through the apparatus, one cathode plate being seen in elevation; Fig. 3 is a longitudinal vertical section through the apparatus; Fig. 4 is a plan of the apparatus, the cover having been removed, and Fig. 5 is a longitudinal vertical section through one end of the apparatus in a somewhat modified form.

Referring to the figures, *a* is the box which is made of any optional suitable material, as iron, or wood coated with lead, or the like; *b* is the conductor supplying current to the anodes. This conductor preferably goes first to a strip *c* of copper on which tin buttons *d* are arranged. To these tin buttons there are strips *e* of tin connected and the anodes *f* are soldered to the latter. On the other side the anodes rest on insulating bars *g*.

*h* are the cathodes which are likewise connected with the conductor *b'* by means of tin strips *e'*, tin buttons *d'* and copper bars *c'*, and they rest on insulating bars *g'* on the opposite side. These anodes *f* and cathodes *h* are suspended alternately in the cells. The content and size of the cells depend on the circumstances of each case. As already mentioned, the thickness of the anodes amounts at the commencement to about 1 to 1½ cm. The distance between the electrodes amounts at the commencement to about 1½ cm; the thickness of the cathodes should be as small as possible.

*i* is a cover for closing the electric cell.

*k* is a steam coil used for heating the electrolyte.

*l* is a siphon for letting off the clear lye, and *m* an opening which is used for drawing off the mud and which can be closed by a plug or the like.

In the form according to Fig. 5 a tap is arranged in place of the siphon *l*. In this case it is arranged that the tap *p* is placed through a socket *o*, and it can be opened or closed by turning the key *q*. Instead of the siphon or tap similar optional suitable means can of course be employed.

The mode of operation with such or similar apparatus is as follows: As anode material Peruvian or Bolivian tin is employed of about the following composition:

|          |          |        |   |
|----------|----------|--------|---|
| Tin      | about 87 | to 93  | % |
| Antimony | " 3      | " 5    | % |
| Arsenic  | " 0.05   | " 5    | % |
| Bismuth  | " 0.1%   |        |   |
| Copper   | " 0.05   | " 0.1  | % |
| Iron     | " 0.2    | " 1.0  | % |
| Silver   | " 0.1    | " 0.15 | % |

105

Traces of gold, sulfur, oxygen, etc.

As already mentioned, plate-shaped anodes are cast of this composition about 1 to 1½ cm. thick as in the electrolytic refining of copper, whereas the cathodes consist of very thin sheets of pure tin. The temperature of the electrolyte is maintained at about 90° C. With a current of 0.9 ampere per square decimeter of electrode surface, the tension between the electrodes amounts to about 0.1 volt. After quite a short time after the circuit has been closed, the cathodes are covered with a metallic compact layer of quite pure tin (99.9% tin), whereas the other metals, as lead, antimony, copper, iron, bismuth, silver, gold, etc., remain behind as anode mud attaching for the most part to the anode. After about 14 days uninterrupted electrolysis, the tension rises to about 0.14 volt. The electrolyte is now drawn off through the above mentioned overflow pipe, and the cathodes as well as the anode residues are removed from the bath. The cathodes may be melted down directly. The anode mud is first scraped off from the anode

120

125

130

residues and then worked up further for obtaining the lead, antimony, silver, bismuth, gold, etc. As some sulfid of sodium is always consumed by oxidation and by the formation of sulfostannate, it is necessary to increase the percentage of sulfid of sodium in the lye again to 10% before commencing the next electrolysis.

Lastly, it is to be noted that the current must not be interrupted during the electrolysis, as otherwise generation of gas at the anodes, impurifying of the cathodes and of the lye etc. occur in consequence of the polarization current.

15. The example which is here given only serves for explaining the mode of working. Under the conditions stated hereinbefore the most favorable results are obtained in practice. It is of course understood that the percentage of sulfid of sodium in the electrolyte and the current density per unit of area of electrode surface can be varied within certain limits having regard to what has been previously stated. For this the percentage of tin 20 in the anode material is decisive, similarly as, for example, in refining copper electrolytically, the percentage of copper of the anode is of influence in the choice of the current density at the electrode.

25. The new method hereinbefore described is at all events up to the present the only one which enables pure, compact and metallic deposits of tin of optional thickness to be obtained electrolytically.

30. What I claim as my invention and desire to secure by Letters Patent is:—

1. The method of obtaining pure tin from

crude tin or tin alloys which consists in electrolytically dissolving the crude tin in a solution of an alkali sulfid and simultaneously 40 plating out the tin upon a cathode of pure tin, and maintaining an electrical tension of less than 0.2 volts between the electrodes.

2. The method of obtaining pure tin from crude tin or tin alloys which consists in electrolytically dissolving the crude tin in a solution of an alkali sulfid and simultaneously 45 plating out the tin upon a cathode of pure tin, maintaining an electrical tension of less than 0.2 volts between the electrodes, regenerating the electrolyte by adding some sulfur thereto and reusing it to electrolyze fresh 50 anodes.

3. The method of obtaining tin from crude tin or tin alloys which consists in treating the 55 impure tin as an anode in an electrolyte composed of an alkaline sulfid solution, depositing the tin upon a cathode having a pure tin surface, maintaining the tension between the electrodes at less than 0.2 volts, and keeping 60 the electrolyte quiescent in order to avoid disturbing the mud deposited in the bottom of the bath, removing the anode residues, regenerating the electrolyte by adding sulfur 65 thereto and reusing it to electrolyze fresh anodes.

In testimony whereof I have signed my name to this specification in the presence of two subscribing witnesses.

OTTO STEINER.

Witnesses:

HEINRICH DIBBEET,  
G. RIVOHNER.